

# United States Patent Office

2,895,859

Patented July 21, 1959

1

2,895,859

## PROCESS FOR THE MANUFACTURE OF PISTON RINGS

Lucien Péras, Billancourt, France, assignor to Régie Nationale des Usines Renault, Billancourt, France

No Drawing. Application June 30, 1955  
Serial No. 519,220

Claims priority, application France August 4, 1954

3 Claims. (Cl. 148—3)

The invention relates to piston rings for internal combustion engines and relates to a process for the manufacture of said piston rings enabling a satisfactory sealing of the combustion chamber to be effected and the wear on said rings to be reduced.

The piston rings of explosion engines or internal combustion engines are currently manufactured by stack moulding in green sand from a cast iron, the average composition of which is: C=3.50%; Si=3.0%; Mn=0.60%; P=0.40%; S=0.05%.

The aim, in this usual manufacture, is for the cast metal to consist of graphite, pearlite and possibly steadiite (phosphorus eutectic Fe—C—P). Every effort is made to avoid cementite, the presence of which would render any machining impossible, and ferrite, a soft constituent, the presence of which is a cause of wear.

The imperative requirements of machining lead to working rules in the foundry which reliably avoid cementite, but in these circumstances it is difficult to avoid ferrite. Slight variations in the casting conditions cause noticeable variations in the proportion of the latter constituent, so that constant supervision is necessary to ensure constancy in the quality of such a product.

The piston rings thus produced have long proved satisfactory in use. They are becoming inadequate, however, even when the desired structure of fine graphite and pearlite is obtained, in the face of the increased requirements of modern engines which are subjected to ever higher loads and rotational speeds.

When conventional piston rings are used in the most modern engines, of cars for example, sealing defects and premature wear appear, which cause a reduction in power and an excessive consumption of lubricating oil.

An important progress is achieved by the present invention, which relates to a method of manufacturing piston rings which makes it possible to achieve an excellent sealing of the combustion chamber, said sealing being maintained during long use of the engine, so that the need for dismantling never arises by reason of deterioration of the piston rings.

According to the invention, the piston rings are obtained by cast iron moulding, the composition of the iron being comprised within the following limits:

|    |              |
|----|--------------|
| C  | 3.00 to 4.00 |
| Si | 1.50 to 3.10 |
| Mn | 0.60 to 1.50 |
| Cu | 0.80 to 2.00 |
| P  | 0.05 to 0.70 |
| S  | 0.02 to 0.15 |

and possibly:

|    |                 |
|----|-----------------|
| Te | 0.000 to 0.050% |
|----|-----------------|

After casting, the parts, which are entirely white in structure, are subjected to a treatment which comprises the following sequence of operations:

(a) Reheating to a temperature at which austenitization takes place and for a time sufficient for all the

2

carbon capable of being dissolved at the temperature in question, to be so. A temperature between 760 and 920° C. is suitable. This heating is followed by quenching, preferably in oil, thus conferring a martensitic structure to the metal. It is also possible to effect a step quenching comprising homogenization at a temperature very slightly above the beginning of the martensitic transformation and short enough in duration to prevent the beginning of any bainitic transformation, then subsequent cooling to produce the martensitic transformation.

(b) A second heating, to bring forth nucleation of the graphite, at a temperature comprised between 420° and 550° C. for a time comprised between 10 minutes and 3 hours.

(c) A third heating, up to a temperature greater than the temperature at the end of the eutectoid transformation, and maintenance at this temperature for the time sufficient and necessary for the carbon in the primary cementite to be entirely graphitized. This heating is followed by cooling, either in still air or in oil, depending on the final hardness desired.

(d) Tempering at a suitable temperature to ensure the desired degree of hardness. For example, when graphitization has been followed by oil quenching, the tempering will be effected at:

600° C. for a desired final hardness of 105 RB  
560° C. for a desired final hardness of 35 RC  
520° C. for a desired final hardness of 38 RC

(e) After these thermal operations, the piston rings are machined and split. A suitable tension is conferred on them by relieving the stresses set up while the ends of the ring are suitably parted. The stress relief is obtained by heating at a temperature slightly less than the tempering temperature or by any other equivalent means.

The piston rings thus obtained are characterized metallographically:

By the absence of primary cementite;

By a distribution of the temper carbon in very fine, very numerous and very regular granules, e.g. 6,000 granules of graphite for mm.<sup>2</sup>;

By a matrix having a very fine sorbitic or pearlitic structure;

By a modulus of elasticity greater by about 50% than that of ordinary grey cast iron. For example, the modulus of elasticity of the piston rings according to the invention has been found to be 18,000 kg./mm.<sup>2</sup>, whereas the modulus of the conventional piston rings of grey cast iron does not exceed 13,000 kg./mm.<sup>2</sup>;

By a higher tensile strength and hardness than those of the usual piston-ring metals. For example, in the piston rings according to the invention, a tensile strength of 80 kg./mm.<sup>2</sup> and a breaking load of 90 kg./mm.<sup>2</sup> are found;

By a remarkable absence of brittleness such as is not found in the usual piston-ring metals;

By a very low coefficient of friction.

A specific example of manufacture of piston rings according to the invention is given below.

After stack casting in green sand, piston rings of cast iron having the composition:

| 65 | C    | Si   | Mn   | Cu   | P    | S    |
|----|------|------|------|------|------|------|
|    | 3.54 | 1.86 | 1.24 | 1.29 | 0.44 | 0.04 |

70 undergo the following series of treatments:

Heating to 810° C., maintenance for 30 minutes at that temperature, then quenching in oil;

Nucleation heating for 2 hours at 450° C.; Graphitization heating for 1 hour at 890° C., then cooling in still air;

Tempering at 600° C., thus obtaining a hardness of from 103 to 104 RB (measured by a ball in the Rockwell machine, load 100 kg.);

Machining, and keeping the ends at the required distance during heating for 5 to 7 minutes at 580° C.;

Grinding to the final dimensions.

The piston rings manufactured as described above ensure a very long period of service. They are particularly valuable in engines in which the cylinder linings are of hard cast iron. In such engines, the wear of the new piston rings is much less (by about 30%) than that of piston rings of conventional manufacture under the same conditions of use. The breakages in service, which occur fairly frequently in very cut-away scraper-rings currently manufactured, never occur with the new piston rings.

1 claim:

1. The process of making alloyed cast piston rings which are substantially free of primary cementite and brittleness, and have a low coefficient of friction, comprising stack molding in a green sand mold the piston rings of a cast iron having the composition 3.00-4.00% carbon, 1.50-3.10% silicon, 0.6-1.5% manganese, 0.8-2.0% copper, 0.05-0.70% phosphorus, 0.02-0.15% sulphur, and the balance substantially all iron, whereby the cast piston rings have a white structure, heating to a temperature slightly above that of the eutectoid transformation point so that austenitization takes place and for a time sufficient for all the carbon to be dissolved, quenching while maintaining a substantially martensitic structure, again heating at a constant temperature between 420° C. and 550° C. for a period of the order of three hours to bring forth graphite nucleation, increasing the temperature after said nucleation heating to a temperature higher than the eutectoid transformation point for a period of time sufficient to graphitize the carbon in the primary cementite, cooling at a controlled rate, said cooling rate being a function of the final hardness to be obtained, and tempering at a predetermined temperature to insure a predetermined hardness.

2. The process of making alloyed cast piston rings which are substantially free of primary cementite and brittleness, and have a low coefficient of friction, comprising stack molding in a green sand mold the piston rings of a cast iron having the composition

|                    |                       |
|--------------------|-----------------------|
| 3.00-4.00% carbon  | 0.05-0.70% phosphorus |
| 1.50-3.10% silicon | 0.02-0.15% sulphur    |
| 0.6-1.5% manganese | 0-0.05% tellurium     |
| 0.8-2.0% copper    |                       |

and the balance substantially all iron, whereby the cast piston rings have a white structure, heating to a temperature slightly above that of the eutectoid transformation point so that austenitization takes place and for a

time sufficient for all the carbon to be dissolved, quenching in oil while maintaining a substantially martensitic structure, again heating at a constant temperature between 420° C. and 550° C. for a period of the order of 3 hours to bring forth graphite nucleation, increasing the temperature after said nucleation heating to a temperature higher than the eutectoid transformation point for a period of time sufficient to graphitize the carbon in the primary cementite, cooling at a controlled rate, said cooling rate being a function of the final hardness to be obtained, tempering at a predetermined temperature to ensure a predetermined hardness, machining the rings and cutting a gap therein to split the rings, stress relieving the rings at a predetermined temperature with the split being set at a predetermined gap opening, said stress relieving temperature being slightly less than the tempering temperature.

3. The process of making alloyed cast piston rings which are substantially free of primary cementite and brittleness, and have a low coefficient of friction, comprising stack molding in a green sand mold the piston rings of a cast iron having the composition

|                 |                  |
|-----------------|------------------|
| 3.54% carbon    | 1.29% copper     |
| 1.86% silicon   | 0.44% phosphorus |
| 1.24% manganese | 0.04% sulphur    |

and the balance substantially all iron, whereby the cast piston rings have a white structure, heating to a temperature of 810° C. and maintaining this temperature for substantially 30 minutes so that austenitization takes place and for all the carbon to be dissolved, quenching in oil while maintaining a substantially martensitic structure, again heating at a constant temperature of 450° C. for a period of two hours to enhance graphite nucleation, graphitization heating at a temperature of 890° C. for 1 hour, cooling in still air at a predetermined rate necessary to obtain a predetermined hardness, tempering at substantially 600° C. for a period of time to obtain a hardness of between 103 and 104 RB when measured by a ball type Rockwell machine with a load of 100 kg., machining the rings and cutting a gap therein to split the rings, stress relieving the rings at a temperature of substantially 580° for a period of between 5 to 7 minutes with the split in the rings being set at a predetermined gap opening, and grinding to final dimensions.

#### References Cited in the file of this patent

#### UNITED STATES PATENTS

|    |           |          |       |                |
|----|-----------|----------|-------|----------------|
| 50 | 2,185,894 | Hultgren | ----- | Jan. 2, 1940   |
|    | 2,214,650 | Bancroft | ----- | Sept. 10, 1940 |
|    | 2,331,886 | Boeghold | ----- | Oct. 19, 1943  |

#### OTHER REFERENCES

The Foundry, April 1949, pages 66-73, 228, 230. Pages 228 and 230 particularly relied on. Transactions, American Society for Metals, preprint No. 32, vol. 47. Manuscript received April 9, 1954.